

## UNITED STATES PATENT OFFICE

2,098,221

## CEMENT OR BINDER MATERIAL

Philip S. Barnhart, Westfield, Mass., assignor to  
 Westfield River Paper Company, Russell, Mass.,  
 a corporation of Massachusetts

No Drawing. Application January 15, 1936,  
 Serial No. 59,308

4 Claims. (Cl. 134—17)

This invention relates to a cement or binder material.

More particularly stated, the invention relates to a cement for uniting or laminating sheets of paper or like material.

The invention has been developed more especially for use in laminating paper sheets of the type known as glassine paper which is semi-transparent. It should be understood, however, that it is not limited to use with this particular type of paper.

Glassine paper is a product made from a highly gelatinized or hydrated fibre obtained chiefly from spruce wood, and processed on a regular Fourdrinier wire machine. The paper after being dried is redampened to give a web with approximately 17 to 25% moisture content. It is then passed through the heated rolls of a super calender to convert it to the semi-transparent stage known as glassine.

Paper, such as glassine paper, when manufactured in relatively heavy weights loses much of its transparency and two light weight sheets when united or laminated by a suitable transparent cement or binder are much more transparent than a single sheet of equivalent weight. This is partially due to the fact that the paper, when finished, has on its surfaces small light marks known as wire marks. When the sheets are laminated by the use of the cement, the surfaces united lose such marks effecting greater transparency.

Paper sheets have been laminated by the use of wax, such as paraffin wax, as a binder, such laminated sheets when subjected to a temperature of approximately 180° F. tend to separate and when subjected to low temperatures the binder tends to become brittle and crack. Obviously, both of these results are detrimental and undesirable.

This invention has for its salient object to provide a cement for laminating sheets of paper or like material, so constituted that it will be effective and will not be rendered ineffective at high or low temperatures.

Another object of the invention is to provide a cement of the character and for the purpose set forth, that can be so used in laminating sheets that the sheets can be joined or united in a simple and economical manner and without undue expense.

Another object of the invention is to provide a cement of the character and for the purpose described that will be relatively transparent.

Another object of the invention is to provide a

cement for the purpose described, so constituted that sheets laminated therewith will be moisture proof.

Further objects will be clear from the following specification.

The invention briefly described consists of a cement compound comprising wax, rosin, rubber and petrolatum. These ingredients when properly proportioned and combined give the desired adhesive quality and produce a moisture resisting 10 or moisture proof binder. Moreover, the cement does not weaken or permit separation of the sheets when subjected to high temperatures, nor does it crack or become less effective at low temperatures.

The wax found most suitable for use is paraffin wax with an approximate melting point of 155° F. This wax has the desired moisture proof or moisture resisting properties, but is not a stable bond at higher temperatures, such as 180°. Sheets joined by wax will separate at such temperatures. Furthermore, the wax is not as flexible at low temperatures and tends to become hard and crystalline causing the sheets to separate very easily.

It was therefore necessary to combine with the wax other ingredients having the desired adhesive qualities to render the cement or bonding material stable and effective at high and low temperatures.

Such ingredients were found in rosin and rubber. The former is fluid when melted and has the desired "tackiness" when mixed with the proper plasticizers.

Rubber gives the cement the desired stability or effectiveness under high and low temperature conditions.

For a plasticizer, petrolatum with a melting point of approximately 125° F. has been found effective.

When a substantially transparent adhesive film is desired, as for instance, for use in uniting or laminating sheets of glassine paper, the grades of ingredients should be chosen with this end in view. Thus, for a semi-transparent cement, 45 rosin, such as "grade X" and rubber in the form or grade of "crepe", or "pale crepe" should be used.

The ingredients found most adaptable for the purpose specified are, therefore, paraffin wax 50 (melting point approximately 155° F.), rosin (grade X, preferred), rubber (preferably "crepe" rubber) and petrolatum (approximate melting point 125° F.).

These ingredients may be combined in the 55

necessary or desired proportions, the proportions that have given the best results being approximately 40-63% wax, 20-45% rosin, 3-12% rubber and 7-13% petrolatum. These proportions may, of course, be varied within limits.

5 Cement or bonding material containing the ingredients mentioned, very effectively fulfill the objects of the invention set forth at the outset of the specification and provides a stable, effective 10 binder, particularly for uniting or laminating paper sheets. The cement is not adversely affected by changes in temperature and is stable and effective at both high and low temperatures.

15 Although certain specified ingredients and approximate proportions have been mentioned in the above specification, it will be understood that there is no intention of limiting the invention to the particular and specified ingredients and proportions, but that applicant is entitled to a reasonable 20 range of equivalents and a reasonable variation in the proportions mentioned, without departing from the spirit or scope of the invention as expressed in the following claims.

What I claim is:

25 1. A cement or binder composed of a mixture of paraffin wax having a melting point of approximately 155° F., rosin, rubber and petrolatum

having a melting point of approximately 125° F., said ingredients being thoroughly intermixed and combined in the following proportions, namely, wax 40-63%, rosin 20-45%, rubber 3-12% and petrolatum 7-13%.

5 2. A cement or binder composed of a mixture of paraffin wax having a melting point of approximately 155° F., rosin, rubber and petrolatum having a melting point of approximately 125° F., said ingredients being thoroughly intermixed and 10 combined in the following proportions, namely, wax 60%, rosin 27%, rubber 5% and petrolatum 8%.

15 3. A cement or binder composed of a mixture of paraffin wax, rosin, rubber and petrolatum, 15 said ingredients being thoroughly intermixed and combined in the following proportions, namely, wax 40-63%, rosin 20-45%, rubber 3-12% and petrolatum 7-13%.

20 4. A cement or binder consisting of paraffin wax 40-63%, rosin 20-45%, rubber 3-12%, and petrolatum in an amount sufficient to produce an adhesive adapted for laminating glassine paper sheets into a laminated sheet which is transparent, moisture-proof and effective at high 25 and low temperatures.

PHILIP S. BARNHART.